

1

3,374,291  
TRITHIOPHOSPHITES OF MERCAPTO  
ACID ESTERS

Herbert Myers, Cherry Hill, N.J., assignor to Mobil Oil  
Corporation, a corporation of New York  
No Drawing. Filed May 25, 1964, Ser. No. 370,112  
6 Claims. (Cl. 260—942)

This invention relates to improved lubricating compositions. More particularly, it relates to a new type of multi-functional additive for such lubricants and a method for their preparation.

It is well known that lubricating compositions are susceptible to oxidation under various conditions of use. For example, oxidation is particularly severe under the high temperature and pressure conditions encountered in internal combustion engines. Such oxidation produces acidic bodies in the lubricating oil which are corrosive to the metal parts of the engine and further results in the deposition of carbonaceous sludge, lacquer and resinous materials whose accumulation impairs the operating efficiency of the engine. In an effort to overcome, insofar as possible, these and other deleterious effects of oxidation it has become the practice to add to the lubricants minor amounts of chemical agents which are commonly known as antioxidants.

It is also the practice to add ingredients to lubricating compositions for the purpose of improving their extreme pressure characteristics, particularly when these compositions are used for lubricating metal surfaces which are subjected to extremely high pressures and high rubbing speeds such as exist in hypoid gears. Such high pressure conditions tend to disrupt the lubricating film with resulting damage to the metal parts to be lubricated. Numerous additives commonly referred to as extreme pressure (E.P.) agents which act to improve the properties of the lubricant under these conditions, are known.

Ordinarily, a combination of antioxidants and E.P. agents must be utilized in lubricating compositions in order to provide the desired effects.

The present invention, however, provides a new class of addition agents which are multi-functional in their activity, i.e., they are capable of improving lubricants in several respects and particularly with regard to oxidation stability and extreme pressure characteristics.

The additives of this invention may be characterized as trithiophosphites of mercapto acid esters. As far as is known, these additive compounds have not been prepared heretofore and they are therefore considered to be new compositions of matter.

It is therefore an object of the present invention to provide certain novel trithiophosphites of mercapto acid esters. A further object is to provide improved lubricating compositions containing these trithiophosphites. Another object is to improve the characteristics, particularly the oxidation stability and E.P. qualities of lubricants by the addition thereto of such trithiophosphites. Other objects of the invention and further advantages thereof will become apparent from the following detailed description.

The trithiophosphites of mercapto acid esters of the present invention may be represented by the general formula,



wherein R is a saturated or unsaturated aliphatic group, aryl group, substituted aliphatic or substituted aryl group containing substituents such as halogens, nitro, cyano, alkyl groups etc.; R' is a saturated or unsaturated aliphatic or cycloaliphatic group, an aryl group, or substituted aliphatic, cycloaliphatic or aryl group containing suitable

2

substituents, e.g., halogens, nitro, cyano, alkyl etc.; and n is an integer from 1 to 3 inclusive.

Some examples of suitable R groups include alkylene groups, such as methylene, ethylene, propylene, butylene, etc.; halogenated alkylene groups, such as chloroethylene; arylene groups or substituted arylene groups, such as phenylene, naphthalene, or phenylene or naphthalene substituted by one or more substituents.

Some examples of suitable R' groups include aliphatic groups, such as methyl, ethyl, propyl, butyl, octyl, oleyl, octadecyl, etc.; substituted aliphatics such as mono- and poly-halogenated alkyds; aryl groups, such as phenyl and naphthyl; and substituted aryls such as phenyl or naphthyls substituted with one or more suitable substituents.

In addition, R' may be a cycloaliphatic group, either unsubstituted or substituted, such as cyclobutyl, cyclopentyl, cyclohexyl, etc.

R preferably contains from 1 to about 40 carbon atoms, the greater number of carbons being generally present when n is more than one; while R' may possess preferably from 1 to about 18 carbon atoms. It will be noted from the general formula that the phosphites may contain from one to three carboxylic acid ester groups depending on the value of n. Compounds containing one or two carboxylic acid ester groups are preferred.

The trithiophosphites of the invention may, in general, be prepared by reacting phosphorus trihalide (PX<sub>3</sub>) with a selected mercapto acid ester in the presence of a suitable base such as tertiary amines, aqueous sodium hydroxide, aqueous sodium carbonate, etc.

The reaction may be illustrated as follows:



wherein R, R' and n have the meanings given above. Various amounts of mercapto acid ester and base may be employed. In general, however, the relative proportions are selected so as to supply at least about 3 mols of base per mol of the phosphorus trihalide.

The reaction is desirably carried out in a non-polar solvent, such as benzene, toluene, isoctane, etc. Although the reaction may be conducted at ambient temperatures, reaction temperatures in the range from about 15 to 50° C. and reaction periods of from about 5 to 15 hours are preferred. The products may be recovered by removing the precipitated base-hydrochloride, such as by filtration, washing the filtrate with 15% hydrochloric acid and water to remove unreacted base, and then topping off the non-polar solvent and unreacted mercapto acid ester.

Exemplary of the trithiophosphites of the invention are those obtained from (a) aliphatic mono-carboxylic mercapto acid esters, and (b) aliphatic polycarboxylic mercapto acid esters and (c) aromatic carboxylic mercapto esters according to the above reaction, and possessing the formula:



where  $x$  and  $y$  represent integers from 1-18. As will be seen from Formula c, the sulfur of the trithiophosphites of the aromatic mercapto esters may be either ortho, meta or para to the carboxylic ester group. In addition, as indicated in the general formula, the aromatic ring of these trithiophosphites may also possess other groups, such as alkyl, halogen, nitro, cyano, etc., attached thereto.

The following examples illustrate the preparation of some typical trithiophosphites of mercapto acid esters.

*Example 1.—Trithiophosphite of butyl thioglycolate—*



Phosphorus trichloride (137 g., 1.0 mole) was added over a period of  $\frac{1}{2}$  hour to a solution of butyl thioglycolate (450 g., 3.1 moles) and triethylamine (312 g., 3.1 moles) in 3.0 liters of benzene while maintaining the reaction temperature at around 15° C. Immediate precipitation of triethylamine hydrochloride occurred. Nitrogen was then introduced and the slurry stirred at 15 to 25° C. for 2 hours and at 50° C. for an additional 3 hours.

The precipitated triethylamine hydrochloride was filtered off and washed with one liter of benzene. Unreacted triethylamine was removed by washing the filtrate with 250 ml. cold 15% hydrochloric acid and 4-500 ml. portions of cold water. After drying the benzene solution over anhydrous potassium carbonate and sodium sulfate, the product was isolated by topping to a pot temperature of 110° C. with nitrogen; to 130° C. under 0.2 mm. pressure and finally filtering through diatomaceous earth.

The resulting product was a clear, pale yellow, viscous liquid which analyzed as follows—

Actual: P, 6.4%; S, 20.8%; Cl, nil. Theoretical: P, 6.5%; S, 20.3%; Cl, nil.

*Example 2.—Trithiophosphite of octyl thioglycolate—*



Following the procedure of Example 1, phosphorus trichloride (68 g., 0.5 mole) was reacted with octyl thioglycolate (350 g., 1.6 moles) and triethylamine (162 g., 1.6 moles) in 2.0 liters of benzene. The product was a viscous, clear pale yellow liquid which analyzed as follows—

Actual: P, 4.6%; S, 15.0%; Cl, nil. Theoretical: P, 4.5%; S, 14.1%; Cl, nil.

*Example 3.—Trithiophosphite of 2-chloroethyl thioglycolate—*



Following the procedure of Example 1, phosphorus trichloride (48 g., 0.35 mole) was reacted with 2-chloroethyl thioglycolate (180 g., 1.13 moles) and triethylamine (115 g., 1.13 moles) in 2.0 liters of benzene. The product was a very viscous, clear, pale yellow liquid which analyzed as follows—

Actual: P, 6.0%; S, 21.1%; Cl, 21.0%. Theoretical: P, 6.3%; S, 19.6%; Cl, 21.7%.

*Example 4.—Trithiophosphite of butyl thipropionate—*



Following the procedure of Example 1, phosphorus trichloride (137 g., 1.0 mole) was reacted with butyl thipropionate (510 g., 3.15 moles) and triethylamine (318 g., 3.15 moles) in 3.0 liters benzene. The product was a pale yellow, clear, viscous liquid that had the following analysis—

Actual: P, 5.8%; S, 19.3%; Cl, nil. Theoretical: P, 6.0%; S, 18.7%; Cl, nil.

*Example 5.—Trithiophosphite of butyl thiosalicylate—*



5

Following the procedure of Example 1, phosphorus trichloride (14 g., 0.10 mole) was reacted with butyl thiosalicylate (69 g., 0.31 mole) and triethylamine (33 g., 0.33 mole) in 500 ml. benzene. The product was a pale yellow, waxy solid that had the following analysis—

Actual: P, 4.2%; S, 14.1%; Cl, nil. Theoretical: P, 4.7%; S, 14.6%; Cl, nil.

*Example 6.—Trithiophosphite of dibutylthiomalonate*



20

Following the procedure of Example 1, phosphorus trichloride (89 g., 0.65 mole) was reacted with dibutylthiomalonate (521 g., 2.0 moles) and triethylamine (202 g., 2.0 moles) in 2.0 liters benzene. The product was a pale yellow, clear viscous liquid that gave the following analysis—

Actual: P, 4.2%; S, 14.1%; Cl, nil. Theoretical: P, 4.7%; S, 14.6%; Cl, nil.

**CATALYTIC OXIDATION TEST**

In order to demonstrate the effectiveness of the compounds of this invention in inhibiting the catalytic oxidation of oil's, the trithiophosphites of the working examples were subjected to a Catalytic Oxidation Test. This test is based on the fact that the oxidized products which form in the oil are known to be acidic in character. Thus, the higher the neutralization number (N.N.), the greater the extent of oxidation. The ability of a compound to maintain the N.N. of an oil composition at a low level is a measure of its antioxidant ability.

According to the test procedure, 25 ccs. of the test oil is placed in a 200 x 25 mm. test tube with 15.6 sq. in. of sand-blasted iron wire, 0.78 sq. in. of polished copper wire, 0.87 sq. in. of polished aluminum wire and 0.167 sq. in. of a polished lead surface. Dry air is passed through the sample at the rate of 10 liters per hour while heating in an aluminum block bath for a period of 24 hours at a temperature of 325° F. The minimum concentration of phosphorus necessary to maintain the acidity of the oxidized oil below a neutralization number of 2 is determined and reported in the following Table I.

It will be seen from Table I that by employing the trithiophosphites of the invention less than 0.10% of phosphorus is required to maintain the neutralization number of the oil below 2.

TABLE I.—CATALYTIC OXIDATION TEST

|         | Trithiophosphite of Example Number | Minimum percent Phosphorus |
|---------|------------------------------------|----------------------------|
| Oil + 1 | 1                                  | 0.082                      |
| Oil + 2 | 2                                  | 0.057                      |
| Oil + 4 | 4                                  | 0.058                      |
| Oil + 5 | 5                                  | 0.084                      |
| Oil + 6 | 6                                  | 0.045                      |

<sup>1</sup> The base oil used was a SAE 10, solvent refined Mid-Continent oil

**SAE LOAD TEST**

The extreme pressure properties of the mercapto acid ester trithiophosphites of the working examples was determined in a SAE load machine. The trithiophosphites were mixed with base oil in amounts sufficient to provide 0.5% by weight of phosphorus. The oil samples are placed in the machine as lubricant for two steel test rings which are rotated at different speeds against each other

in the same direction while a gradually increasing load is mechanically applied. The machine is operated at a rubbing ratio of 14.6 to 1 and a shaft speed of 500 r.p.m. and the test is continued until seizure occurs. The results are reported in Table II. It will be seen that the oil containing no additive fails during the "break in" period. By contrast, the oils containing the compounds of the invention exhibit superior E.P. characteristics as indicated by the heavy loads necessary to produce seizure.

TABLE II.—SAE LOAD TEST

| Trithiophosphite of Example No. | Phosphorus Cont. (Wt. percent) | SAE Load Test, 500 r.p.m.<br>Seizure Load |
|---------------------------------|--------------------------------|-------------------------------------------|
| Oil 1                           | 0.5                            | 460+, 460+                                |
| Oil 2                           | 0.5                            | 460+, 460+                                |
| Oil 3                           | 0.5                            | 410, 460+                                 |
| Oil 4                           | 0.5                            | 400, 415                                  |
| Oil 5                           | 0.5                            | 390, 390                                  |

<sup>1</sup> The base oil used was a SAE 90, solvent refined, Mid-Continent Oil.

<sup>2</sup> Fails break in. Break in=20 pounds.

The trithiophosphites of this invention are effective in improving the characteristics particularly the oxidation stability and E.P. characteristics of a variety of lubricants including lubricating oils, greases, hydraulic fluids etc. These lubricants may contain either mineral or synthetic base oils. Thus, mineral oils from various crudes, both solvent and acid refined, hydrocracked, etc., as well as synthetic hydrocarbons, including olefin polymers, hydrogenated olefin polymers, alkyl benzenes, etc., synthetic esters, such as di-2-ethylhexyl sebacate, dialkyl adipate, trimethylol propane dioctanoate, etc., silicone fluids and the like may have their characteristics improved by the addition of the trithiophosphites described herein.

The amount of trithiophosphite added to the lubricant will depend on various factors, including the type of the lubricant the presence or absence of other ingredients, the extent of oxidation stability desired, etc. In general, the trithiophosphites are employed in amounts from about 0.1 to about 10, preferably from about 0.5 to about 5 weight percent.

The lubricating compositions of the present invention may, of course, also contain effective quantities of various other materials which are normally used therein such as detergents, inhibitors, V.I. improvers, thickening agents, defoamants, supplemental antioxidants or E.P. agents, etc.

It will, of course, be appreciated that many variations and modifications may be practiced without departing from the scope and spirit of the present invention.

Having thus described the invention, what I desire to obtain and secure by Letters Patent is:

1. A mercapto acid ester trithiophosphite of the formula



wherein R is selected from the class consisting of alkylene, alkenylene, arylene, alkarylene and aralkylene having from 1 to about 40 carbon atoms; R' is selected from the class consisting of alkyl, cycloalkyl, alkenyl, aryl, alkaryl, aralkyl, and monochloroalkyl and having from 1 to about 18 carbon atoms; and n is an integer of from 1 to 3, and when R' is alkyl, R is selected from the class consisting of alkenylene, arylene, alkarylene and aralkylene.

15 2. A trithiophosphite according to claim 1 of the formula:



20 where x is an integer from 1 to about 18 wherein R' is selected from the class consisting of alkenyl, aryl, alkaryl, aralkyl and monochloro alkyl.

3. A trithiophosphite according to claim 1 of the formula:



30 4. A trithiophosphite according to claim 1 of the formula:



where x and y are integers from 1 to about 18.

5. A trithiophosphite of 2-chloroethyl thioglycolate.

40 6. A trithiophosphite of butyl thiosalicylate.

#### References Cited

#### UNITED STATES PATENTS

2,824,847 2/1958 Fath ----- 260—942 X

CHARLES B. PARKER, Primary Examiner.

F. M. SIKORA, A. H. SUTTO, Assistant Examiners.